

Jan. 11, 1927.

W. H. SPENCER

1,614,263

METHOD FOR MAKING ORNAMENTAL PANELS, SIGNS, AND THE LIKE

Filed March 18, 1926

*Fig. 1.*



*Fig. 4.*



*Fig. 2.*



*Fig. 5.*



*Fig. 3.*



*Fig. 6.*



*Fig. 12.*



*Fig. 7.*



*Fig. 11.*



*Fig. 8.*



*Fig. 10.*



WITNESS

*O. H. Holmes*

BY *Knight Bz*  
ATTORNEY

## UNITED STATES PATENT OFFICE.

WILLIAM H. SPENCER, OF BOGOTA, NEW JERSEY, ASSIGNOR TO I. P. FRINK INC., OF NEW YORK, N. Y., A CORPORATION OF NEW YORK.

## METHOD FOR MAKING ORNAMENTAL PANELS, SIGNS, AND THE LIKE.

Application filed March 18, 1926. Serial No. 95,694.

This invention relates to the formation of designs, legends, or the like upon suitable bases or backgrounds to form ornamental panels, signs, etc., such, for example, 5 as the ornamental signs shown in United States Patent No. 1,525,107 which was granted in my name under date of February 3, 1925.

The primary object of my invention is to provide certain details of refinement in 10 methods for producing ornamental signs, panels, and the like, and as exemplified in my above identified patent, contemplates an illuminated sign constructed on a base of glass or other translucent material.

15 One of the objects of my present invention is to provide an improved process for electroplating portions of an ornamental sign, panel or the like, which portions surround or lie contiguous to other portions 20 which are not electroplated.

Certain specific objects of invention will appear in the specification and be pointed out in the appended claims, reference being had to the accompanying drawings which 25 show a preferred embodiment of my invention, and in which:—

Figure 1 is a fragmentary cross-section of a permanent base which may be constructed of plate glass or any other suitable material; 30 Figure 2 is a similar fragmentary cross-section of said base after a sheet of resist or masque has been applied thereto;

Figure 3 is a similar fragmentary section showing portions of the resist or masque cut 35 away to roughly conform to the design or legend to be produced on the sign;

Figure 4 is a similar fragmentary section of the partly-finished sign after superficial portions of the plate glass have been removed by some suitable agency such, for example, as sand-blast or hydrofluoric acid, to conform to the design or legend to be produced;

Figure 5 is a fragmentary cross-section 45 similar to Figure 4 showing the application of a conductive layer preparatory to an electro-deposit of metal;

Figure 6 is a similar fragmentary cross-section showing the partly-finished sign 50 after a flash deposit of electroplating;

Figure 7 is a fragmentary cross-section of the partly-finished sign after the removal of those portions of the preliminary conductive layer and superimposed flash deposit which

cover the untouched original surface of the 55 glass;

Figure 8 shows a fragmentary cross-section of the finished sign according to one of the adaptations of my invention shown on the drawings;

Figure 9 is a plan view of the finished panel or sign;

Figure 10 is a fragmentary cross-section of the partly-finished sign according to a modification of the process subsequently to 65 the stage shown in Figure 5;

Figure 11 is a fragmentary cross-section of the finished sign according to this modified adaptation of my invention.

Figure 12 is a fragmentary cross-section 70 of the completed sign or panel according to another embodiment of my invention.

According to the embodiment of my invention shown in Figures 1 to 9 of the drawings, a permanent base 1 which may 75 be constructed of plate glass or other suitable material, is prepared for having portions of its surface roughened by the application of a sand-blast or other suitable agency, by covering it with a masque or

resist 2 as shown in Figure 2. After portions of this resist or masque have been cut away to correspond to the design or legend to be produced, as indicated at 3 in Figure 3, the base 1 is immersed in hydrofluoric acid or exposed to a sand-blast whereby exposed portions of said base are excavated as indicated in Figure 4. According to this adaptation of my invention, this 85 operation forms a roughened background 4

extending around and contiguous to raised portions 5 of base 1 which raised portions remain due to the protection afforded them by the residual portions of the resist or masque. As shown in Figure 5, a conductive 90 layer 6 is applied to the roughened surface and extended in such a way as to cover the resist or masque portions 2. For this

purpose, a graphite solution or a coat of metallic paint such as that referred to in 100 my above identified patent, may be utilized

to form a permanent conductive layer on the roughened portions 4 of the base and an integral extension thereto over the residual portions of the resist or masque. The 105 partly finished sign thus produced is next

immersed in an electrolytic bath to receive a flash deposit 7 of electroplating as indicated

in Figure 6. The residual portions of the resist or masque above the raised portions 5, are then removed together with the flash deposit of metal superimposed thereon, as indicated in Figure 7, this operation being performed according to the present adaptation of my invention in such a way as to leave a projecting fin or ridge 8 of electrically conductive material as shown in Figure 10. It will be understood from this description that when the partly-finished sign or panel in the form shown in Figure 7 is placed in an electrolytic bath, the electro-deposition of metal will produce a metal layer 9 with a relatively heavy raised border 9<sup>a</sup> along the fin or ridge 8 and around the edges of the design or legend. This process produces a pronounced ornamental border of great beauty as shown in Figures 8 and 20 9 of the drawings.

Referring now to Figures 5, 10, and 11 of the drawings, my invention contemplates a modification in the above process, according to which the residual portions of the masque 2 together with the superimposed portions of the conductive layer shown in Figure 5, are cut away flush with the original surfaces of the raised portions 5, thus leaving the partly-finished sign or panel in 25 the form shown in Figure 10. The subsequent electroplating operation according to this procedure, may thus be made to produce a border of greater finish due to the better defined edge of the conductive layer left by 30 the sharply defined cut made in removing portions of the conductive layer as originally applied.

Referring now to the embodiment of my invention shown in Figure 12, the process 40 described above in connection with Figures 1 to 9 inclusive, has been applied to the production of an ornamental panel having a base or block 10 which has been excavated by sandblast or other agency to receive a 45 conductive coating 11 with a superimposed flash deposit of electroplating. Prior to the deposition of the main layer 12 of electroplating, the layers of conductive coating and flash deposit have been cut away in such a 50 manner as to leave an upwardly-presented ridge 13 which during the final electroplating operation, produces a pronounced ornamental border 14 which in this instance extends around the electroplated area as indicated in Figure 12.

My improved method as described above 55 may be advantageously employed for the production of signs, ornamental panels, grilles, etc.

In the manufacture of signs, wherein the letters are usually made transparent or translucent, the metal may be deposited upon the background.

For ornamental plates where the field is 65 usually made transparent or translucent, the

metal may be deposited in the plate to form the design.

I claim:

1. The method of forming signs, which method consists in forming a permanent base, in forming roughened surfaces contiguous to a design or legend to be produced, in applying a conductive layer to the roughened areas as well as to the areas corresponding to said design or legend, in electroplating said conductive layer, and finally in removing those portions of the conductive and electroplated layers superimposed upon said design or legend. 75

2. The method of forming signs, which method consists in forming a protective covering over those portions of a permanent base corresponding to the design or legend to be produced, in removing portions of the superficial areas of said base to form roughened surfaces contiguous to said design or legend, in applying a conductive layer to the roughened areas as well as to the protective covering superimposed upon said design or legend, in electroplating said conductive layer, and finally in removing said protective covering together with the conductive coating and electro-deposited layer superimposed upon said design or legend. 85

3. The method of forming signs, which method consists in forming a protective covering over those portions of a permanent base corresponding to the design or legend to be produced, in removing contiguous portions of said base, in applying a conductive layer to the protective covering of said design or legend and to the surface left by the removal of said base portions, in removing said protective covering together with its superimposed portion of the conductive coating, and finally, in electroplating the remainder of the sign covered by the conductive layer. 95

4. The method of forming signs, which method consists in forming a protective covering over those portions of a permanent base corresponding to the design or legend to be produced, in removing contiguous portions of said base, in applying a conductive layer to the protective covering of said design or legend and to the surface left by the removal of said base portions, in imparting to said conductive layer a flash electro-deposit of metal, in removing said protective covering together with that portion of the conductive coating and flash-deposit superimposed thereupon, and finally, in electroplating the remainder of the sign covered by the conductive layer. 115

5. The method of forming signs, which method consists in preparing a permanent base with portions of the superficial area thereof roughened to correspond to the design or legend to be produced, in applying a conductive layer to the roughened and un- 125

roughened areas of said base, in electrolytically depositing a metallic layer over the entire area of said conductive layer, in removing the portions of said conductive layer 5 which lie above the unroughened areas together with the corresponding portions of the electro-deposited layer of metal, and in continuing the electroplating process on the electroplated roughened areas until the desired thickness is obtained.

6. The method of forming a device of the character described, which method consists in forming a permanent base, in forming a design or legend on said permanent base, in applying a conductive layer to the surface of said base, in electro-plating said conductive layer, and finally, in removing portions of the conductive layer with superimposed electroplating to conform to the design or 20 legend to be produced.

7. The method of forming an ornamental panel, which method consists in forming said panel with smooth and roughened areas

corresponding to the ornamental design to be produced thereon, in applying a conductive 25 coating over the entire superficial surface of said areas, in electroplating said conductive coating over its entire superficial area and in removing the portions of the electroplated conductive coating overlying the 30 smooth areas whereby a sharply defined border line is formed around those portions of the electroplated coating overlying the roughened areas.

8. The method of forming an ornamental 35 panel, said method consisting in forming a permanent base, in applying a conductive layer to the surface of said base, in electroplating said conductive layer, in removing portions of the conductive layer with corresponding portions of the superimposed electroplated layer, and finally in continuing the electroplating process on the unremoved portions of the electroplated conductive layer 40 until the desired thickness is attained.

WILLIAM H. SPENCER.